

## UNITED STATES PATENT OFFICE

2,039,524

AGENTS RENDERING TEXTILE MATERIALS  
FAST TO CREASING

Alfred Eckelmann and Ernst Koch, Frankfort-on-the-Main-Hochst, Germany, assignors to General Aniline Works, Inc., New York, N. Y., a corporation of Delaware

No Drawing. Application November 2, 1934,  
Serial No. 751,254. In Germany November 9,  
1933

7 Claims. (Cl. 134—18)

The present invention relates to agents rendering textile materials fast to creasing and to a process of treating textile materials with said agents.

We have found that textile, such as, for instance, viscose artificial silk or cotton, may be rendered fast to creasing by treating them with solutions or emulsions of salts of imido ethers and of salts of amidines or derivatives thereof and aldehydes or substances yielding aldehyde and then heating them to temperatures of about 50° C. to about 120° C. The aldehydes may be used in the form of solutions or, in case of low molecular aldehydes, in the form of gases. The textiles may be treated first with solutions of salts of imidoethers and amidines and then with aldehydes. But it is also possible to treat the textiles first with the aldehydes and then with the solutions of the salts of imidoethers and amidines. Furthermore, the aldehydes or the substances yielding aldehydes may be introduced into the solutions or emulsions of the salts of imidoethers and amidines and the textiles may be treated with the solutions or emulsions thus obtained.

As salts of such imidoethers there may be mentioned, for instance: stearimidoethylether hydrochloride, stearimidoobutyletheroxalate, laurimido-chloroethylether hydrochloride, oxystearimido-butylether hydrochloride, abietimidoethylether hydrochloride, acetimidostearylether hydrochloride, benzimidododecylether hydrochloride, the reaction product of sebacyldinitrile with 2 mols of butanol and HCl or the product which is obtainable by causing the nitrile of a naphthenic acid to react with ethylalcohol in the presence of HCl.

As amidines there may be used, for instance, stearamidine hydrochloride, lauramidineformate, the amidine which is obtainable from stearimido-ethylether by reaction with ethylene diamine, abietamidine hydrochloride, laurdiethylamidine acetate.

The mixtures of imidoethers and amidines may consist of mixtures of pure imidoethers and pure amidines as well as of mixtures of imidoethers and amidines obtained from mixtures of technical acids by way of the respective nitriles or from imidoethers hydrochlorides, respectively.

As such mixtures there may be used besides those mentioned in the examples: the mixtures consisting of the imidoethylether hydrochloride of technical stearic acid and the amidine hydrochloride of technical stearic acid, furthermore, the mixture of imidoethylether hydrochloride of

palm nut oil fatty acid and the amidine of technical stearic acid.

As aldehydes there may be mentioned: formaldehyde, acetaldehyde, glyoxal, and as substances yielding aldehydes: dimethylol urea and dimethylol formamide.

The solubility and the stability of the solutions of certain of the salts of these imidoethers or amidines may be enhanced by using during the preparation of the solutions simultaneously emulsifying or dispersing agents or protective colloids. As such agents there may be mentioned, for instance, the salts of the amides carrying sulfo or carboxyl groups or the esters of higher fatty acids, salts of urethanes carrying sulfo or carboxyl groups, fatty alcohol sulfonates, water-soluble oxethylated fatty alcohols, oxethylated fatty amines, oxethylated esters or amides of higher fatty acids, carbohydrates, oxethylated or other water-soluble albuminous substances and similar water-soluble high-molecular substances or mixtures of the said substances.

The advantage of the present process resides in the fact that the textile fibers need only be heated to a temperature of at most 120° C. so that the fiber is not detrimentally affected and the tissue is prevented from becoming yellow. The textile fabrics treated according to the present process are, furthermore, distinguished by a very soft feel.

The following examples serve to illustrate the invention but they are not intended to limit it thereto; the parts are by weight:

(1) Viscose fabric is steeped with 1000 parts of a formaldehyde solution of 20% strength which contains 10 parts of stearimidoethylether hydrochloride and 10 parts of stearamidine formate (both produced with the aid of technical stearic acid). After hydroextracting, the material is dried at about 90° C. It is then very fast to creasing and has an agreeable soft feel.

Instead of the hydrochloride of stearimidoethylether there may also be used the hydrochloride or oxalate of the imidomethylether or imidobutylether obtainable from coconut fatty acid nitrile.

(2) 5 parts of stearimidoisobutylether hydrochloride, 5 parts of stearamidine formate and 3 parts of the ammonium salt of polyvinylbutyl-ethermaleic acid are dissolved in 1000 parts of formaldehyde solution of 20% strength. Mixed fabric of viscose and natural silk is treated with this solution, then squeezed and dried at about 100° C. The fabric now has a very good fastness to creasing and a very soft feel.

- (3) Linen tissue is introduced into a bath which contains per liter 25 parts of imidobutyl-ether hydrochloride, obtainable from the fatty acid nitrile of coconut oil and 20 parts of stearic amidine formate. After squeezing, the material is passed through a formaldehyde solution of 20% strength, hydroextracted and dried at 90° C. to 100° C. The material has become fast to creasing and is distinguished by a full handle.
- (4) In 1 liter of formaldehyde solution of 20% strength there are dissolved 20 parts of imidoethylether hydrochloride, obtainable from technical stearic acid, and 6 parts of the amidine, obtainable by causing the said hydrochloride to react with ethylenediamine, and viscose artificial silk tissue is treated with this solution at ordinary temperature. The material is squeezed, centrifuged and dried at 100° C.; it is then pretty fast to creasing and possesses an agreeable soft feel.
- (5) Cotton tissue is handled for 10 minutes in a solution of 15 parts of myristimidoamylether hydrochloride of the formula



30 and 10 parts of lauridiethylamidine acetate of the formula



35 in 1 liter of water. The tissue is hydroextracted and then hung up in a chamber filled with formaldehyde vapor; after half-an-hour it is dried on a calendar at 100° C. The cotton tissue then proves to be fast to creasing to a great extent and possesses a soft feel.

(6) Mixed fabric consisting of wool and viscose artificial silk is treated with a solution which contains per liter 120 parts of dimethylol urea, 45 10 parts of laurimidohexylether hydrochloride of the formula



and 10 parts of the amidine which is obtained by causing ethylene diamine to react with the imidoethylether hydrochloride obtainable from the fatty acid nitrile of palm nut oil. Thereupon, 55 the tissue is centrifuged and dried at about 110° C. It has become very fast to creasing and retains this property after being washed.

We claim:

1. The process which comprises treating a textile material with an aqueous preparation containing an addition salt of an imidoether, an addition salt of an amidine and an aldehyde and 5 drying the material at a temperature of about 50° C. to about 120° C.

2. The process which comprises treating a textile material with an aqueous preparation containing an addition salt of an imidoether, an addition salt of an amidine and formaldehyde and 10 drying the material at a temperature of about 50° C. to about 120° C.

15 3. The process which comprises treating a textile material with an aqueous preparation containing formaldehyde, the imidoethylether hydrochloride, obtainable from the technical stearic acid and the amidine hydrochloride which is obtainable by converting this imidoethylether hydrochloride by means of ethylenediamine, and drying the material at a temperature of about 50° C. to about 120° C.

20 4. The process which comprises treating a textile material with an aqueous preparation containing dimethylol urea, laurimidohexylether hydrochloride of the formula



25 and the amidine hydrochloride, obtainable by causing ethylene diamine to react with the imidoethylether hydrochloride which is obtainable from the fatty acid nitrile of palm nut oil.

30 5. Agents for treating textile material comprising an addition salt of an imidoether and an addition salt of an amidine:

35 6. An agent for treating textile material comprising the imidoethylether hydrochloride, obtainable from the technical stearic acid, and the amidine hydrochloride, obtainable by converting this imidoethylether hydrochloride by means of ethylenediamine.

40 7. An agent for treating textile material comprising dimethylol urea, laurimidohexylether hydrochloride of the formula



45 and the amidine hydrochloride, obtainable by causing ethylene diamine to react with the imidoethylether hydrochloride which is obtainable from the fatty acid nitrile of palm nut oil.

50 ALFRED ECKELMANN.  
ERNST KOCH.